

## UNITED STATES PATENT OFFICE

2,189,970

METHOD OF MAKING GLASS TO METAL  
SEALS

Stanton Umbreit, West Orange, N. J., assignor, by  
mesne assignments, to Radio Corporation of  
America, New York, N. Y., a corporation of  
Delaware

No Drawing. Application October 30, 1937,  
Serial No. 172,055

2 Claims. (CL 49—81)

My invention relates to glass to metal seals, particularly to the manufacture of metal alloys which have predetermined coefficients of thermal expansion and which will readily seal with glass.

5 In sealing glass to metal, it is desirable to select the glass and the metal with coefficients of thermal expansion which substantially coincide or match over the entire temperature range from room to glass softening temperature. Cobalt-  
10 nickel-iron alloys of the type disclosed in the U. S. patent to Burger and Hull, 2,071,196, February 16, 1937, have expansion characteristics which adapt them for sealing with commercial boro-silicate glass. It has been found, however, 15 that in commercial production of these alloys the expansion characteristics of the alloys may vary within limits and render sealing with a given glass difficult. When an alloy of this kind is formed by pressing or drawing into the desired 20 shapes, such as small thin walled cylinders or eyelets for sealing with glass, it appears to vary in crystal or grain structure and in coefficient of expansion.

An object of my invention is to make glass to 25 metal seals in which the coefficient of thermal expansion of the glass and the metal match throughout the temperature range from room to sealing temperature of the glass.

A further object of my invention is to make 30 a stable alloy which will not change in crystal or grain structure, and which has a coefficient of thermal expansion such that it will seal readily with commercial glasses.

An alloy in extensive commercial use for sealing with glass, and consisting of about 18% cobalt, 30% nickel, and the remainder iron when first alloyed appears to consist of austenite. This alloy when drawn into thin walled eyelets and annealed appears under the microscope to have the 35 regular twinned polygonal crystals similar to the gamma phase of iron. It has been found, however, that when this alloy is drawn and is also cooled to a temperature of about 0° C. the crystal structure suddenly changes, the shape of crystals being irregular and the individual grains being needle-like and resembling martensite or the alpha phase of iron. When this transformation 40 of crystal structure occurs, the body of the alloy suddenly expands. The coefficient of thermal expansion of the cobalt-nickel-iron alloy in the gamma phase may be about  $4.5 \times 10^{-6}$  per degree C., whereas after the transformation, the coefficient of thermal expansion may be of the 45 order of  $8$  to  $9.5 \times 10^{-6}$  per degree C. This trans-

formation may in some cases occur at temperatures between 0° C. and +50° C.

The alloy in the austenitic state when cooled several hundred degrees from an elevated temperature contracts rapidly, at a rate of about 5  $16 \times 10^{-6}$  centimeters per centimeter per degree C., and at a temperature of between 400 and 500° C. the rate of contraction is reduced to about 10  $3.5 \times 10^{-6}$  centimeters per centimeter per degree C. As the cooling continues to about 0° C., the austenitic state of the alloy abruptly changes to 15 the martensitic state with an actual increase in volume. Further cooling continues contraction at the rate of about  $9 \times 10^{-6}$  centimeters per centimeter per degree C. If the metal is now heated, it 20 expands at the rate of  $9 \times 10^{-6}$  until a temperature of 500° C. is reached, when the martensite gradually changes to austenite with a decrease in volume. It appears that at temperatures above about 700° C., the alloy is in the austenitic state 25 irrespective of its crystal or grain structure below that temperature. According to my invention, the temperature at which the alloy may change from the austenitic to the martensitic state is lowered to a temperature below any temperature 30 encountered in manufacture or use so that the alloy retains its coefficient of thermal expansion 35 of  $3.5 \times 10^{-6}$  below sealing temperature.

According to my invention, the temperature at 40 which the austenitic alloy is transformed or changed into martensitic alloy is lowered to a point well below temperatures encountered in manufacture or use of the alloy. By adding about .05% or more carbon to the solid solution of the alloy, the transformation temperature may be 45 lowered to below -200° C., the crystal structure of the alloy becomes stable, and eyelets drawn from the alloy retain a constant coefficient of thermal expansion and seal readily with glass.

A boro-silicate glass, commercially known as 50 "hard glass," with a coefficient of thermal expansion of about  $4.5 \times 10^{-6}$  per degree C. comprises 65% silica ( $SiO_2$ ), 23% boro-oxide ( $B_2O_3$ ), 7% sodium oxide ( $Na_2O$ ), and 5% aluminum oxide ( $Al_2O_3$ ) and may be advantageously sealed to 55 my improved alloy comprising 18% cobalt (Co), 28% nickel (Ni), 54% iron (Fe), and about .05% carbon in solid solution with the alloy. The alloy may comprise by weight from 45% to 54% iron, 28% to 30% nickel and 18% to 25% cobalt. The thermal expansion characteristic of this glass and alloy is substantially uniform at about 4.5  $\times 10^{-6}$  from below room to sealing temperature.

While the specific example of glass and alloy 55

- 5 matching in thermal expansion characteristics has been given, it will be apparent to those skilled in the manufacture of glass to metal seals that changes in the glass may be made to change its coefficient of thermal expansion and that corresponding changes may be made in the alloy to bring the thermal expansion characteristics into coincidence.

10 I prefer, according to one embodiment of my invention, to prepare an alloy of cobalt, nickel, and iron in the proportions above mentioned and to form sealing members or bodies such as cylinders or eyelets from sheets of the alloy. The sealing bodies are then treated, according to my invention, by diffusing into the bodies pure carbon preferably by carburizing the parts at a high temperature. Good results have been obtained by heating eyelets of the cobalt-nickel-iron alloy in an atmosphere of hydrogen with a graphite block for 30 minutes at 1100° C. Alternatively, the eyelets may be heated in hydrogen containing hydro-carbons such as xylene or light oil to diffuse carbon throughout the body of the eyelets. I have also found that a convenient way to introduce carbon into the eyelets is to immerse the eyelets in molten sodium cyanide for 10 minutes at 800° C.

15 20 25 While the .05% carbon content in the iron-nickel-cobalt alloy mentioned reduces the transformation temperature of the alloy to a safe low value, the carbon content may, if desired, be greater. The greater the carbon content, the

lower is the transformation temperature. The amount of carbon diffused into the alloy, however, is limited by the presence of carbon on the sealing surface of the alloy bodies. According to a further feature of my invention, I introduce 5 an excess of carbon or saturate the alloy with carbon and then remove the carbon at the sealing surface of the alloy body by heating in an atmosphere of wet hydrogen.

10 I claim:

1. The method of sealing a glass with a predetermined coefficient of thermal expansion to a metal body of predetermined shape of an alloy of 45% to 54% iron, 28% to 30% nickel and 18% to 25% cobalt, comprising working said alloy 15 to form the body of said shape, diffusing carbon through said body at an elevated temperature to lower the temperature of transformation of the alloy from the austenitic to the martensitic state and, placing said glass in contact with said body, 20 and heating to the sealing temperature.

2. The method of sealing a glass with a predetermined coefficient of expansion to a pre-formed metal body of an alloy of iron, nickel, and cobalt, comprising working the alloy to form said 25 body, heating said body in the presence of carbonaceous gas to introduce more than .05% carbon into said alloy, removing the carbon on the surface of said body, and placing said glass in contact with said body and heating to sealing 30 temperature.

STANTON UMBRETT.